

# United States Patent [19]

Kin et al.

[11] Patent Number: 4,626,485

[45] Date of Patent: Dec. 2, 1986

[54] SUBSTITUTED SQUARIUM COMPOUNDS, PROCESS FOR PREPARING THE SAME AND ELECTROPHOTOGRAPHIC PHOTORECEPTORS CONTAINING THE SAME

[75] Inventors: Seki Kin; Hiroyuki Tanaka; Satoshi Saeki; Kaoru Torikoshi; Lyong S. Pu, all of Kanagawa, Japan

[73] Assignee: Fuji Xerox Co., Ltd., Tokyo, Japan

[21] Appl. No.: 733,165

[22] Filed: May 13, 1985

[30] Foreign Application Priority Data

May 11, 1984 [JP] Japan ..... 59-92764  
May 25, 1984 [JP] Japan ..... 59-104776

[51] Int. Cl. 4 ..... G03G 5/06; G03G 5/14

[52] U.S. Cl. ..... 430/59; 430/58;  
430/73; 564/307

[58] Field of Search ..... 430/58, 59, 73;  
564/307

[56]

## References Cited

### U.S. PATENT DOCUMENTS

|           |         |                   |          |
|-----------|---------|-------------------|----------|
| 3,824,099 | 7/1974  | Champ et al. .... | 430/58   |
| 4,353,971 | 10/1982 | Chang et al. .... | 430/58   |
| 4,486,520 | 12/1984 | Yanus ....        | 430/73 X |
| 4,523,035 | 6/1985  | Yanus ....        | 564/307  |
| 4,524,219 | 6/1985  | Law ....          | 564/307  |
| 4,524,220 | 6/1985  | Law ....          | 564/307  |
| 4,525,592 | 6/1985  | Law et al. ....   | 564/307  |

### OTHER PUBLICATIONS

Loutfy et al, "Photoconductivity of Organic Particle Dispersions: Squaraine Dyes", P.S.E., vol. 27, No. 1, Jan./Feb. 1983, pp. 5-9.

Primary Examiner—Roland E. Martin  
Attorney, Agent, or Firm—Sughrue, Mion, Zinn,  
Macpeak, and Seas

[57]

## ABSTRACT

Novel squaraine compounds which have a flat photo-sensitivity in the wide range from visible ray region to the near infrared ray region as a charge generator and which can be prepared by reacting squaric acid and an aniline derivative, and electrophotographic photoreceptors containing the squaraine compounds are disclosed.

13 Claims, 2 Drawing Figures



U.S. Patent

Dec. 2, 1986

4,626,485

FIGURE 1



FIGURE 2



SUBSTITUTED SQUARIUM COMPOUNDS,  
PROCESS FOR PREPARING THE SAME AND  
ELECTROPHOTOGRAPHIC PHOTORECEPTORS  
CONTAINING THE SAME

FIELD OF THE INVENTION

This invention relates to novel squarium compounds having a flat photosensitivity in the wide range from visible ray region to the near infrared ray region as a charge generator, a process for preparing them and electrophotographic photoreceptors containing the squarium compounds.

BACKGROUND OF THE INVENTION

Hitherto, inorganic photographic materials such as amorphous selenium, selenium alloys, cadmium sulfide and zinc oxide and organic photographic materials represented by polyvinylcarbazole and polyvinylcarbazole derivatives are widely known as electrophotographic photoreceptors.

It is well known that amorphous selenium or selenium alloys have superior properties as electrophotographic photoreceptors and have been put into practice use. However, in producing these materials, a complicated vacuum deposition process is necessary, and further the vacuum-deposited film obtained has a disadvantage in that the film lacks flexibility. Zinc oxide is used as a dispersed photographic material in which zinc oxide is dispersed in a resin, but such material has a problem such as a low mechanical strength and cannot be used repeatedly as is.

Polyvinylcarbazoles known as organic photoconductive materials have advantages such as transparency, good film-forming property and flexibility, but polyvinylcarbazoles per se have no photosensitivity in at visible ray region, an cannot be used practically alone. Accordingly, various sensitization methods have been proposed therefor. Although a spectral sensitization of polyvinylcarbazole using a sensitizing dye has resulted in expanded spectral sensitivities extending to visible ray region, a sufficient photographic sensitivity as electrophotographic photoreceptors cannot be obtained, and it still has a drawback that a photo-fatigue is remarkable.

On the other hand, a spectral sensitization with an electron acceptor gives rise to electrophotographic photoreceptors having a sufficient photosensitivity, and some of them has been practically used. However, there are still more problems on mechanical strength and durability.

Various extensive studies have been made on photosensitive materials and there are many reports. However, electrophotographic photoreceptors having a superior electric characteristic and a sufficient photosensitivity have not yet been obtained. At present, there are reports about phthalocyanines which show superior electrophotographic characteristics as dispersed photosensitive materials. However, their spectral sensitivity is partial to long wavelength region, and they have a drawback that reproduction of red color is inferior.

SUMMARY OF THE INVENTION

An object of this invention is to provide novel squarium compounds having a flat photosensitivity in the wide range from the visible ray region to the near infrared ray region, a process for preparing squarium

compounds and electrophotographic photoreceptors containing such squarium compounds.

Another object of this invention is to provide photoconductive materials having an extremely high photosensitivity, which are possible to use in every electrophotographic process and have a spectral sensitivity in the range from the visible ray region to the near infrared ray region.

A further object of this invention is to provide extremely superior electrophotographic photoreceptors having a flexibility that inorganic photographic materials fail to have, which are free from drawbacks of organic photographic materials such as polyvinylcarbazole-trinitrofluorenones, that is a low abrasion resistance and lack of mechanical strength, and which are superior in mechanical strength such as abrasion resistance and have a flat spectral sensitivity in the wide range from visible ray region to the near infrared ray region.

As a result of extensive studies to obtain photoconductive materials having improved properties over conventional inorganic photographic materials, organic photographic materials or organic dispersed photographic materials, having superior electrophotographic properties and flexibility, and further having high photographic sensitivity in the wide range from visible ray region to the near infrared ray region, the present inventors found that the squarium compounds represented by the following general formula (I) possess extremely superior characteristics:



wherein X represents a hydrogen atom, a fluorine atom, a chlorine atom, a bromine atom, a nitro group, or a cyano group.

BRIEF DESCRIPTION OF THE DRAWINGS

FIGS. 1 and 2 are profile sections of compositions of electrophotographic photoreceptors of this invention.

In figures, "1" shows an electroconductive support, "2" shows a charge generation layer, "3" shows a charge transport layer and "4" shows a photosensitive layer.

DETAILED DESCRIPTION OF THE INVENTION

The squarium compounds of this invention represented by formula (I) above can be prepared by reacting 3,4-dihydroxy-3-cyclobutene-1,2-dione (hereinafter referred to as squaric acid) represented by formula (II):



with an aniline derivative of formula (III):



and then recrystallizing the compound from an appropriate solvent.

Examples of the squarium compounds of formula (I) above of this invention include the following compounds.

| Compound No. |
|--------------|
| (1)          |
|              |
| (2)          |
|              |
| (3)          |
|              |
| (4)          |
|              |
| (5)          |
|              |
| (6)          |
|              |

wherein X has the same meaning defined for formula (I) above.

In formula (I), X preferably represents a hydrogen atom, a fluorine atom, or a chlorine atom.

The reaction of squaric acid of formula (II) with an aniline derivative of formula (III) can be carried out by heating squaric acid and the aniline derivative in an inert organic solvent, such as n-butyl alcohol, amyl alcohol, or a mixed solvent of n-butyl alcohol or amyl alcohol with benzene, toluene or xylene, at about 120° C. to about 140° C. for about 3 hours to about 5 hours. The resulting compound can be purified by washing

60 The spectral sensitivity of the squarium compounds of this invention show a flat photosensitivity in the range of from 400 to 850 nm, and the squarium compounds of this invention have a sufficient photosensitivity in the range from the entire visible ray region to the near infrared ray region.

65 The squarium compounds of formula (I) can be used in electrophotographic photoreceptors having a multi-layer structure. That is, in electrophotographic photoreceptors having a double layer structure consisting of a charge generation layer and a charge transport layer, a combination of the charge generation layer containing a squarium compound of this invention and a known

charge transport layer comprising a photoconductive polymer such as polyvinylbibenzothiophene, polyvinylpyrene, polyvinylanthracene, or a polyvinylcarbazole or a layer containing triallylpyrazoline, triphenylmethane, oxadiazole, tetraphenylbenzidine, or trinitrofluorenone in a binder resin results in the improvement of chargibility of electrophotographic photoreceptors, lowering of residual potential, and further the improvement of mechanical strength.

As shown in FIGS. 1 and 2 which explain the construction of electrophotographic photoreceptor of this invention having a double layer structure, a photosensitive layer 4 which is composed of a lamination of charge generation layer 2 containing a squarium compound of this invention and a charge transport layer 3 containing a charge transport material is provided on an electrically conductive support 1. The thickness ratio of the charge generation layer to the charge transport layer is preferably from about  $\frac{1}{2}$  to about 1/200. Further, the squarium compound and a charge transport material may be incorporated into one layer to form a single-layered photoreceptor, if desired.

The charge generation layer can consist of a squarium compound alone or a combination of the squarium compound and a binder resin. The ratio of the squarium compound of formula (I) to the binder resin used is from about 10% by weight to about 90% by weight, preferably from about 10% by weight to about 50% by weight.

A solvent coating method and a vacuum evaporation method can be used to prepare the charge generation layer with the squarium compound of this invention without using a binder resin.

The film thickness of charge generation layer is from about  $0.1\mu$  to about  $3\mu$ , preferably from  $0.2\mu$  to  $1\mu$ .

For the purpose of its dispersion in a binder, the compound may be ground into fine particles by a known method using any conventional mill, such as an SPEX MILL, ball mill or RED DEVIL (trade name). Particle size of the pigment is generally not more than  $5\mu$ , preferably 0.01 to  $3\mu$ , but the particle size is not limited thereto.

The binder used in the charge generation layer may have or may not have photoconductivity. Examples of binders having photoconductivity include photoconductive polymers such as polyvinylcarbazole, polyvinylcarbazole derivatives, polyvinylnaphthalene, polyvinylanthracene, polyvinylpyrene, or other organic matrix materials having a charge transport property.

Moreover, known insulating resins which have no photoconductive property can be used as binders. Examples of such insulating resins include polystyrene, polyesters, polyvinyltoluen, polyvinylanisole, polychlorostyrene, polyvinyl butyral, polyvinyl acetate, polyvinylbutyl methacrylate, copolystyrene-butadiene, polysulfone, copolystyrene-methyl methacrylate and polycarbonates.

In order to improve mechanical strength of the electrophotographic photoreceptors obtained, a plasticizer can also be used as in the case of ordinary polymeric materials. Examples of plasticizers which can be used include chlorinated paraffins, chlorinated biphenyl, a phosphate plasticizer and a phthalate plasticizer. These plasticizers can be used in an amount of 0 to 10% by weight based on the weight of the binder used without adversely affecting the photosensitivity and electrical

properties of the electrophotographic photoreceptors thereby improving the mechanical properties.

The binder having dispersed therein a squarium compound is coated on an electroconductive support. The coating can be performed by a conventional method such as dip method, spray method, bar coater method and applicator method. A good photosensitive layer can be obtained by any of the above methods.

Usable electrically conductive supports include metals (e.g., aluminum, nickel, chromium, iron, stainless, copper, etc.), paper which is rendered electrically conductive, as well as polymeric films and glass plates having an electrically conductive coat of the above metals, Au, Ag, indium oxide, indium tin oxide, etc.

A surface layer such as a protective layer and an insulating layer may further be provided on the photosensitive layer so as to prevent mechanical damage and chemical change in properties of the photosensitive layer. The protective layer is a layer having low electric resistance of  $10^8$  to  $10^{14}$   $\Omega\text{cm}$  which can be used in so-called Carlson process, and the insulating layer is an electrically insulating layer which can be used in a process as described in U.S. Pat. Nos. 3,041,167 and 3,438,706. Both layers are substantially transparent to light for exposure and the thicknesses of the protective layer and the insulating layer are about 2 to  $20\mu$  and about 10 to  $40\mu$ , respectively.

In order to prevent injection of electron from an electrically conductive support to the photosensitive layer, a barrier layer may be formed between the support and the photosensitive layer. For the purpose, aluminum oxide, nylon, epoxy resins can be used. Such a barrier layer may not be formed when the photoreceptor is used in the process of U.S. Pat. Nos. 3,041,167 and 3,438,706 as described above or when the charge transport layer is formed as a lower layer on the support in the preparation of double-layered photoreceptor (FIG. 2). An adhesive layer may also be formed between the support and the photosensitive layer to improve adhesion therebetween.

The electrophotographic photoreceptor of the present invention may be used not only with ordinary copiers but also when laser printers, as well as intelligent copiers since the photoreceptor of the present invention is sensitive to laser. Laser which can be applied to the photoreceptor of the present invention is preferably a semiconductor laser such as those of Ga-As type semiconductors (e.g., Ga-As, Al-Ga-As, Ga-As-P, etc.).

The squarium compounds of formula (I) of this invention can be applied to various materials such as optical recording media (e.g., laser disk) and organic solar batteries, in addition to the electrophotographic materials.

This invention will now be explained in more detail by the following examples.

#### EXAMPLE 1

##### Preparation of Compound (1)

5.76 g of N-benzyl-N-methyl-m-hydroxyaniline and 1.48 g of squaric acid were heated on an oil bath kept at 130° to 140° C. in a mixed solvent of 70 ml of n-butyl alcohol and 20 ml of benzene with stirring for 3 hours, whereby greenish crystals were precipitated. After cooling, the crystals were collected by filtration, washed with methanol, and then dissolved in propylamine, followed by reprecipitating from water to obtain 5.0 g (76.3% yield) of the desired squarium compound.

Decomposition point: 293° C. to 295° C.



a charge transport layer and a charge generation layer containing said squarium compound.

3. An electrophotographic photoreceptor as claimed in claim 2, wherein said charge transport layer comprises a photoconductive polymer selected from the group consisting of polyvinylbibenzothiophene, polyvinylpyrene, polyvinylanthracene and polyvinylcarbazole.

4. An electrophotographic photoreceptor as claimed in claim 2, wherein said charge transport layer comprises a compound selected from the group consisting of triarylpazoline, triphenylmethane, oxadiazole, tetraphenylbenzidine or trinitrofluororenone and a binder resin.

5. An electrophotographic photoreceptor as claimed in claim 2, wherein said charge generation layer is comprised substantially of said squarium compound.

6. An electrophotographic photoreceptor as claimed in claim 2, wherein said charge generation layer comprises said squarium compound in an amount of from about 10 to 90 weight percent based on the weight of said charge generation layer.

7. An electrophotographic photoreceptor as claimed in claim 6, wherein said squarium compound is present

in an amount of from about 10 to 50 weight percent based on the weight of said charge generation layer.

8. An electrophotographic photoreceptor as claimed in claim 2, wherein said charge generation layer is from about 0.1 to 3 micron thick.

9. An electrophotographic photoreceptor as claimed in claim 8, wherein the thickness ratio of said charge generation layer to said charge transport layer is from about  $\frac{1}{2}$  to about 1/200.

10. An electrophotographic photoreceptor as claimed in claim 2, wherein said charge generation layer is present between said support and said charge transport layer.

11. An electrophotographic photoreceptor as claimed in claim 2, wherein said charge transport layer is present between said support and said charge generation layer.

12. An electrophotographic photoreceptor as claimed in claim 1, wherein said photosensitive layer comprises a layer containing said squarium compound and a charge transport material.

13. An electrophotographic photoreceptor as claimed in claim 2, wherein said squarium compound is dispersed in the form of particles in said charge generation layer.

\* \* \* \* \*